

# UNITED STATES PATENT OFFICE.

WILLIAM BRACKMANN, OF NEWARK, NEW JERSEY, ASSIGNOR TO THE OCEAN LEATHER CO., INC., OF NEW YORK, N. Y., A CORPORATION OF DELAWARE.

## PROCESS OF SHRINKING SHARK-SKINS.

1,304,256.

Specification of Letters Patent.

Patented May 20, 1919.

No Drawing.

Application filed November 2, 1918. Serial No 260,898.

To all whom it may concern:

Be it known that I, WILLIAM BRACKMANN, a citizen of the United States, residing at 56 Fabyan Place, Newark, State of New Jersey, have invented certain new and useful Improvements in Processes of Shrinking Shark-Skins, of which the following is a specification, reference being had therein to the accompanying drawing.

10 This invention relates to the shrinking of skins, more particularly shark skins, and it has for its object primarily to produce shrunken grain.

15 In carrying out my invention I employ a solution consisting substantially of

Gambier, 2 lbs., boiled and strained.  
Muriatic acid,  $\frac{1}{2}$  lb.

Oxalic acid, 2 oz.

Aluminum-chlorid,  $\frac{1}{10}$  of an oz.

20 Water, 3 gallons.

I mix these ingredients thoroughly and then make the solution luke-warm, and apply to the skins, in any suitable manner, as by a brush, giving the skins a good coat.

25 I then put the coated skins on a table or tables, or other support, of glass, metal or wood greased, or some analogous slippery support, so that the skins will not stick thereto. The skins are then placed in a dry-  
30 ing room and subjected to a temperature of not more than 110° Fahrenheit, for a suitable length of time.

Practical tests have proven that skins thus

treated produce the desired shrunken grain and that the quality of the skin is not impaired, but, on the other hand, is greatly improved.

35 While the proportions above specified are what I have found to produce most satisfactory results, the proportions may be varied 40 within certain limits without departing from the spirit of the invention or sacrificing any of its advantages.

45 The skins are to be left in tan for from four to five days, and then taken out, treated with my solution, and afterward further tanned. In contradistinction to pickling the skins in a pickling solution, in a revolving drum, or a pickling vat, I place the skins, when partially tanned, on a flat surface and 50 apply my solution to the grain side with a brush or sponge. This treatment causes the grain to draw or shrink, thereby producing a shrunken grain, or a natural embossing.

55 What is claimed as new is:—

1. The process of treating skins to produce shrunken grain, which consists in treating them with a luke-warm solution containing gambier and then drying the same in a temperature not greater than 110° Fahrenheit.

2. Material for treating skins embodying gambier, muriatic acid, oxalic acid and aluminum-chlorid.

60 In testimony whereof I affix my signature.

65 WILLIAM BRACKMANN.